

# UNITED STATES PATENT OFFICE.

MAX HELBIG, OF FREDRIKSSTAD, NORWAY.

## PROCESS FOR THE EXTRACTION OF SULFUR FROM METAL SULFIDS.

1,315,496.

Specification of Letters Patent.

Patented Sept. 9, 1919.

No Drawing.

Application filed April 15, 1919. Serial No. 290,271.

To all whom it may concern:

Be it known that I, MAX HELBIG, of Fred-  
riksstad, in the Kingdom of Norway, have  
invented certain new and useful Improve-  
ments in Processes for the Extraction of  
Sulfur from Metal Sulfids; and I do hereby  
declare the following to be a full, clear,  
and exact description of the invention, such  
as will enable others skilled in the art to  
10 which it appertains to make and use the  
same.

The invention relates to the treatment of  
sulfid ores or other metal sulfids with the ob-  
ject of obtaining sulfur and has for its ob-  
15 ject a process by means of which metal  
phosphid is obtained as a by product.

According to the hitherto known processes  
the extraction of the sulfur contained in  
metal sulfids such as for instance the iron  
20 sulfid  $FeS_2$  (iron pyrite) is connected with  
such difficulties that they cannot be practi-  
cised with economical advantage on a com-  
mercial scale.

The present invention now has for its  
25 object a process by which these difficulties  
are avoided.

This process allows of extracting the sul-  
fur of the sulfids in an elemental state at  
the same time as the metal sulfids are con-  
30 verted into technically valuable phosphids  
for instance ferro-phosphorus ( $Fe_2P$ ).

To obtain this result a charge consisting  
of the sulfid in question, a phosphate as well  
as fluxing materials and carbonaceous re-  
35 ducing material is melted down. The compo-  
sition of the charge as well as tempera-  
ture and other conditions are so controlled as  
to cause the phosphorus of the phosphate  
40 to combine with the metal of the sulfid to  
form phosphid while the sulfur is liberated.

When iron pyrite is treated the process  
may be carried out as follows:

Iron pyrite in which the principal con-  
stituent is the iron sulfid  $FeS_2$  is mixed with  
45 apatite, coke and quartz in proportions so  
calculated as to correspond to the equation:



One third of the sulfur will be distilled off  
solely by the action of the heat. The rest of 50  
the sulfur is expelled as a result of the  
reaction between the components of the  
charge.

In the described manner it is possible by  
the use of a quantity of pyrite corresponding 55  
to 100 parts b. w. of  $FeS_2$  to obtain about 53  
parts b. w. of sulfur 53 parts b. w. of ferro-  
phosphorus with a content of 21 per cent.  
of phosphorus.

The process is suitably carried into effect 60  
in closed furnaces preferably electrically  
heated, which are connected with suitable  
purification and condensation devices for  
the escaping sulfur vapors.

Metal phosphid and slag is tapped off pe- 65  
riodically or continuously.

I claim:

1. Process for the extraction of sulfur  
from metal sulfids consisting in heating with  
a charge containing the metal sulfid a phos- 70  
phate as well as a silicious flux and carbo-  
naceous reducing material so proportioned  
as to cause the phosphorus of the phos-  
phate to combine with the metal of the sul-  
fid, while the sulfur of the sulfid escapes 75  
with the gaseous reaction products.

2. Process for the production of sulfur  
from metal sulfids, which consists in heating  
a mixture of the sulfid with calcium phos- 80  
phate, a silicious flux, and carbon so propor-  
tioned as to cause the entire phosphorus of  
the phosphate to combine with the metal of  
the sulfid to form a phosphid, the entire sul-  
fur of the sulfid escaping in the form of ele- 85  
mental sulfur.

In testimony that I claim the foregoing  
as my invention I have signed my name in  
presence of two subscribing witnesses.

MAX HELBIG.

Witnesses:

AUGUST BRIGGE,  
OLGA MÜLLER.